

T. A. ZELLERS.  
MANUFACTURE OF GLASS.

No. 66,274.

Patented July 2, 1867.



Witnesses:

*W.D. Lewis.*

*EB.Cushing.*

Inventor:  
Theodore A. Zellers,

by Bakewell & Christy,  
his attorneys.

# United States Patent Office.

THEODOR A. ZELLERS, OF EAST BIRMINGHAM, PENNSYLVANIA.

*Letters Patent No. 66,274, dated July 2, 1867.*

## IMPROVEMENT IN MANUFACTURE OF GLASS.

The Schedule referred to in these Letters Patent and making part of the same.

### TO ALL WHOM IT MAY CONCERN:

Be it known that I, THEODOR A. ZELLERS, of East Birmingham, in the county of Allegheny, and State of Pennsylvania, have invented a new and useful Improvement in the Manufacture of Window-Glass; and I do hereby declare the following to be a full, clear, and exact description thereof, reference being had to the accompanying drawings, making a part of this specification, in which—

Figure 1 is a vertical section, formed by a plane passing through the flattening-oven in the line  $z-z$ , fig. 2.

Figure 2 is a horizontal section, formed by a plane passing through the line  $y-y$ , fig. 1; and

Figure 3 shows in perspective the apparatus by which I use, as fuel, oils and oily products and compounds.

Like letters of reference in the different figures designate like parts.

In the manufacture of window-glass the molten glass is usually blown into the shape of a hollow cylinder, which is then cut or fractured lengthways, so as to be spread out, when sufficiently heated, into a flat sheet.

My invention relates to an improved furnace for flattening such glass, and consists in treating such glass cylinders by the application of the heat evolved in the combustion of hydrocarbon oils or their products or compounds, and in the construction of apparatus for burning such oils, in connection with a furnace or oven fitted with suitable devices for handling and flattening the glass.

To enable others skilled in the art to make and use my invention, I will proceed to describe its construction and mode of operation.

$a$  is the flattening-oven, covered by the arch  $a'$  and enclosed by walls of any convenient material, shape, or mode of construction. Through a door or opening in the front wall I introduce the glass cylinders successively, either by a car,  $b$ , or place them in the oven on a raised platform in lieu of the car  $b$ ; the upper face of either the car or platform being concave, as shown in fig. 1, the better to receive the glass cylinder. As shown in the drawings, the car  $b$  rests on a revolving platform or turn-table,  $c$ , so that, carrying the glass cylinder, it may be brought to the position it is shown to occupy in fig. 2, either by its handle,  $b'$ , or by a lever,  $c''$ , attached to the standard  $c'$ , which supports the turn-table  $c$ .  $d$  is the flattening-car, having a perfectly flat surface, its top usually of stone, on which the glass cylinder is smoothed out into a flat sheet when sufficiently heated, and by which it is borne back through a door or aperture,  $e$ , in the rear wall of the flattening-oven  $a$  to a tempering-oven,  $f$ , of the ordinary construction, where it receives further treatment in the usual or any known way. The car  $d$  is moved back and forth by power communicated through a shaft,  $g$ , and pinion,  $g'$ , to the toothed rack  $d'$  attached to the car  $d$ . The burning apparatus which I employ consists of a trough or box,  $h$ , furnished with two or more supply pipes—one,  $l$ , for the admission of water, and another,  $l'$ , for the admission of oil, benzine, gasoline, or other hydrocarbon or product or compound thereof, inflammable at a comparatively low temperature, and lighter than water. In order to guard against danger of accident, I cause the water pipe  $l$  to discharge its contents higher up in the trough  $h$  than the oil pipe  $l'$ . I thus keep the mouth of the latter continually covered with water, so as to prevent all possibility of the fire passing back through the pipe  $l'$  to the reservoir, or otherwise endangering life or property. The oil or oily product or compound thus introduced spreads over the surface of the water, where it is readily ignited, and continues burning till the supply is either cut off or exhausted. Since such liquids as those above named require for their complete and perfect combustion a considerable quantity of oxygen, I provide for such want by intermingling any desirable quantity of atmospheric air with the products of the combustion of the oil, introducing the air for that purpose through pipes  $i$  inserted in the bottom of the trough  $h$ . The upper ends of such pipes  $i$  are even with or a little above the surface of the burning oil, which is kept at a uniform level by carrying off the superfluous water, if any there be, by a small waste pipe,  $m$ . In this way the quantity of oxygen requisite to secure the complete combustion of the oil is secured, so that all or nearly all the carbon of the oil or oily fluid employed, which would otherwise pass off in the shape of smoke, is converted into heat, and, passing up through the flattening-oven  $a$ , is directly applied to heating the glass on the flattening-car  $d$ . The superfluous products of combustion pass off through the chimneys  $n$ , where the draught is regulated by one or more dampers,  $n'$ , in each.

After the car  $b$ , with the glass cylinder resting thereon, is brought to the position shown in fig. 2, the operator introduces his tool or "cropper" through an opening in the front wall of the furnace, carefully lifts the cylinder therefrom, places it on the car  $d$ , where, with the usual tools, he spreads it out, as it becomes

softened by the heat from the burning oil. As soon as it has been properly flattened, it is passed back into the tempering-oven *f*, as already stated, removed from the car *d*, and subjected to the usual treatment. The car *d* is returned to the flattening-oven *a*, and the operation repeated with each successive cylinder. In that part of the process of making window-glass to which my invention particularly relates, the fuel heretofore generally employed usually contains more or less sulphur, which, as the fuel is consumed, passes off in a gaseous state, and, coming in contact with the glass, materially lessens its transparency, and produces what is called "sulphured" or "smoked glass." Also, the draught which supports the combustion, when coal or coke is employed for fuel, invariably carries with it into the furnace more or less dust, usually of the ashes of combustion. This dust settles on the flat surface of the top of the car *d*, and when the glass is flattened down, and is in a plastic condition, it produces irregularities in the surface of the glass, known among window-glass makers as "pimples." By treating the glass in the manner described, with the heat evolved in the combustion of hydrocarbon oils or their products or compounds, I avoid both of the practical difficulties above suggested. Such oils are usually free from sulphur or sulphurous compounds, so that the glass is not at all liable to injury thereby, and the combustion of such oils producing no ash, and the products of combustion being wholly consumed, the flattening-oven *a* is wholly free from dust, smoke, or other deleterious matter of a similar character. Another advantage which I secure is a better application of the heat. In such furnaces or ovens a somewhat rapid draught or current of heated air is required, in order that the glass cylinder may be raised to the desired temperature without unduly heating the flat stone which usually forms the top of the car *d*. If a high heat be applied directly to the stone, or if a dead heat be kept up in the oven, the stone is liable to become so highly heated as partially to melt the glass thereon while it is being flattened, in which case the glass settles into the pores of the stone, and produces a defective quality of window-glass known as "burnt" glass. Also, by supplying oxygen, and securing a perfect combustion of the carbon contained in the fuel employed, I economize fuel, and save the waste of carbon which attends the process of coking bituminous coal, which is now done in order to prepare it for such uses. And further, by my invention I utilize benzine, gasoline, and other products of the distillation of crude petroleum, which are of little or no commercial value; or I use the crude petroleum itself, whereby I effect a great saving in the cost of the fuel. By the use of the cocks *o o* I regulate the supply of oil and water, or cut off such supply altogether, and by the dampers *n' n'* I increase or lessen the draught, and thereby regulate the application of the heat to the glass. In connection with the devices described, I sometimes use a furnace of the ordinary construction, which I place immediately under the fire-box *h*, and in such case make the fire-box *h* removable. Then, if so preferred, when about to heat up the oven *a*, (an operation which requires about twelve hours,) I remove the fire-box *h*, heat up the oven *a*, by burning the fuel usually employed for such purposes, in the ordinary way, and, when the oven is properly heated, replace the fire-box *h*, and proceed thereafter substantially in the manner above described. The heat from such furnace may then be employed to perfect the combustion of the oil or oily products or compounds. In order to secure cheapness of construction and convenience in handling, I usually make the box or trough *h*, air pipes *i i*, and supply and waste pipes *l l' m* of cast iron, and cast them solid in one piece. The pipes *l l'* may be coupled with the pipes leading to the reservoirs in any convenient way, so as readily to be uncoupled for the purpose of removing the box *h*. By the use of the turn-table *c* or vibratory car *b*, I secure another desirable result. If the pole or "cropper" of the operator, when he is about to lift the glass cylinder from the car *b* to the flattening-stone, be passed into the cylinder otherwise than in a line parallel with the axis of the cylinder, the pole, first coming in contact with the cylinder at one end, frequently causes the edges of the cylinder, where cut or fractured preliminary to its being flattened out, to slip past each other, and lap one on the other from one-eighth to half an inch, more or less. The edges solapping will not be acted on by the heat to the same extent as the remainder of the cylinder, whereby is caused an unequal expansion of the different parts of the glass, which commonly results in the cylinder or sheet becoming utterly worthless. It has been observed also that the edges solapping contract dampness between them, which facilitates greatly the unequal action of the heat, and consequently aids materially in spoiling the glass. By my invention, the cylinder is turned with one end toward the opening in the front wall of the oven, through which the operator passes in his pole or cropper in a line direct, or nearly so, with the axis of the cylinder, brings the cropper in contact with the inside of the cylinder throughout its entire length, and removes it to the flattening-stone, without causing or giving rise to the danger of injury above suggested. In this way I save a considerable percentage of the loss which occurs in the manufacture of window-glass. In burning the oils named, and applying the heat evolved thereby to the uses above set forth, I do not limit myself to any particular form of fire-box or burning apparatus, provided only a perfect or nearly perfect combustion of the oil is secured, but I consider the form of box described to be especially adapted to the purpose above set forth.

What I claim as my invention, and desire to secure by Letters Patent, is—

1. Treating glass cylinders in a flattening-oven, and reducing them to flat sheets, by the heat evolved from the combustion of hydrocarbon oils, or their products or compounds, substantially in the manner and for the purposes hereinbefore set forth.
2. In connection with an oven for flattening glass, the car *b* and turn-table *c*, or a raised vibratory platform in lieu thereof, for the purpose of so turning glass cylinders as to enable the operator, standing in front of the flattening-car, to insert his cropper in such cylinders, in a line with the axis of each such cylinder, substantially in the manner and for the purposes above set forth.

In testimony whereof I, the said THEODOR A. ZELLERS, have hereunto set my hand.

THEODOR A. ZELLERS.

Witnesses:

A. S. NICHOLSON,  
Geo. H. CHRISTY.